

[54] GALLIUM ARSENIDE PHOTOCATHODE

[75] Inventor: Martin Pion, Harlow, England

[73] Assignee: International Standard Electric Corporation, New York, N.Y.

[22] Filed: Jan. 30, 1974

[21] Appl. No.: 438,139

|           |         |                       |           |
|-----------|---------|-----------------------|-----------|
| 3,575,628 | 4/1971  | Word .....            | 313/95    |
| 3,592,705 | 7/1974  | Kawashima et al ..... | 148/187   |
| 3,631,303 | 12/1971 | Antypas et al .....   | 148/171 X |
| 3,823,043 | 7/1974  | Andre et al .....     | 148/171   |

Primary Examiner—G. Ozaki

Attorney, Agent, or Firm—John T. O'Halloran, Menotti J. Lombardi, Jr., Edward Goldberg

[30] Foreign Application Priority Data

Feb. 6, 1973 United Kingdom ..... 5782

[52] U.S. Cl. ..... 148/171; 148/172; 148/173; 357/30; 313/95; 250/213

[51] Int. Cl. 2 ..... H01L 7/38

[58] Field of Search ..... 148/171-173; 357/30; 313/95; 250/213

[56] References Cited

UNITED STATES PATENTS

3,478,213 11/1969 Simon et al ..... 357/30

[57]

ABSTRACT

A gallium arsenide photocathode is formed from a substrate of gallium arsenide on which are grown a first thin gallium aluminum arsenide layer and a further thin active layer of gallium arsenide. A coating of wax is applied over the thin active GaAs layer and around the sides and peripheral edges of the structure. A central region of the GaAs substrate is then etched to expose the inner GaAlAs layer while leaving a supporting rim around the edges. The rim permits use of a thinner GaAlAs layer.

4 Claims, 1 Drawing Figure



PATENTED AUG 26 1975

3,901,745



## GALLIUM ARSENIDE PHOTOCATHODE

## BACKGROUND OF THE INVENTION

## 1. Field of the Invention

This invention relates to gallium arsenide photocathodes of the transmission type in which light may be directed upon one side of the device in order to produce photon-excited electron emission from the opposite side.

## 2. Description of the Prior Art

The upper limit to the thickness of a GaAs wafer that can be used as a transmission type photocathode is set by the short diffusion length of photon excited electrons in GaAs (typically 10  $\mu\text{m}$  or less). The mechanical properties of GaAs make it difficult if not impossible to produce satisfactory self-supporting wafers of the requisite thickness. One method of overcoming this problem involves growing the wafer on a supporting substrate of GaAlAs which is itself grown on a seed of GaAs. At some stage of manufacture the GaAs seed material is removed by lapping, for if this were not done its optical absorption would prevent the completed structure from being used in the transmission mode. The GaAlAs layer will have to be quite thick, typically 150 to 300  $\mu\text{m}$ , in order to provide a sturdy support for the GaAs layer. This requires the maintenance of comparatively tight manufacturing tolerances during the growth stage in order to produce a homogeneous uniform thickness layer of such depth. The present invention is concerned with the provision of a rim structure which will provide a measure of mechanical support for the photocathode at its periphery.

A prior art semiconductor device with a supporting rim structure is shown in U.S. Pat. No. 3,478,213, issued Nov. 11, 1969. This, however, is used in an electron multiplier of different materials.

## SUMMARY OF THE INVENTION

It is therefore the primary object of the present invention to provide an improved semiconductor photocathode structure and method.

According to the invention there is provided a method of making a GaAs transmission type photocathode including the steps of growing an epitaxial layer of GaAlAs upon a GaAs substrate, of growing an epitaxial layer of GaAs upon the layer of GaAlAs, and of removing, without penetrating through either of the epitaxial layers, the central region of the GaAs substrate to form an apertured rim supporting the periphery of the layers. This permits use of a thinner GaAlAs layer, typically in the range of 40 to 100  $\mu\text{m}$ .

There follows a description of the manufacture of a transmission type photocathode embodying the invention in a preferred form.

## BRIEF DESCRIPTION OF THE DRAWINGS

The single FIGURE schematically shows a cross-section through the photocathode.

## DESCRIPTION OF THE PREFERRED EMBODIMENTS

Referring to the drawing, a layer 1 of p-type  $\text{Ga}_{0.5}\text{Al}_{0.5}\text{As}$ , typically 40 to 100  $\mu\text{m}$  thick, is grown by liquid epitaxy upon a GaAs substrate 2 which is at least 150

$\mu\text{m}$  thick. (The preferred orientation of the GaAs substrate is the 100 crystal orientation, an alternative preferred orientation is the 111 crystal orientation). Next

the GaAlAs layer 1 is covered with a thin active outer layer 3 of p<sup>+</sup> type GaAs typically 5 to 10  $\mu\text{m}$  thick. The coated substrate is prepared for etching by attaching it to a support 4 by bedding it face downwards in wax 5. Further wax is painted round the rim 6 of the back of the substrate so that when the support is immersed in

10 an etching solution only the central region 7 of the back of the substrate is exposed to the etch. The width of the masked peripheral region 6 is typically 1 to 2 mm.

The central region of the GaAs 7 substrate is next removed chemically by a bubble etching technique which permits uniform removal over a large area. The coated substrate, still secured to its support 4, is placed with its epitaxially grown layers face upwards in a suitable etch contained in a vessel with a porous base through which is pumped nitrogen gas. The exposure of the GaAlAs layer can be seen by inspection of the substrate as it is slightly different in color, and hence it is not necessary to use a GaAs only selective etch. A suitable non-selective etch is a mixture of sulphuric acid and hydrogen peroxide. The lattice constants of GaAs and GaAlAs are closely matched to provide an improved layered structure of higher sensitivity and reduced stress.

Conventional bonding techniques are used for making electrical contact with these devices, such contact being made either directly to the grown layer 3 or to the rim of the supporting substrate 2. The exposed surface of the GaAs layer 3 may be subjected to conventional caesiating treatment used to improve efficiency by lowering the work function.

It is to be understood that the foregoing description of specific examples of this invention is made by way of example only and is not to be considered as a limitation on its scope.

## What is claimed is:

1. A method of making a GaAs transmission type photocathode comprising the steps of growing an epitaxial layer of GaAlAs upon a GaAs substrate, growing an epitaxial layer of GaAs upon the layer of GaAlAs, coating the entire outer surface of the GaAs epitaxial layer with a layer of wax extending around the sides of the GaAs epitaxial and GaAlAs epitaxial layers and around the peripheral rim portion on the opposite surface of the GaAs substrate so that only the central region of the substrate is exposed, and removing the exposed central region of the GaAs substrate without penetrating through either of the epitaxial layers to form an apertured rim of GaAs supporting the periphery of the GaAlAs and GaAs layers.

2. The method of claim 1 including the step of attaching the wax-coated outer surface to a support.

3. The method as claimed in claim 2 wherein the central region of the GaAs substrate is removed by etching 60 to expose the GaAlAs layer.

4. The method as claimed in claim 3 and including removing the layer of wax and caesiating at least a portion of the outer surface of the GaAs layer.

\* \* \* \* \*